

# UNITED STATES PATENT OFFICE.

LUCIUS A. KINGKINNEY, OF CENTRALIA, WASHINGTON, ASSIGNOR TO WILLIAM A. CARLISLE, OF ONALASKA, WASHINGTON.

## BRIQUET AND BINDER FOR THE SAME.

1,359,074.

Specification of Letters Patent. Patented Nov. 16, 1920.

No Drawing.

Application filed May 12, 1920. Serial No. 380,888.

To all whom it may concern:

Be it known that I, LUCIUS A. KINGKINNEY, a citizen of the United States, residing at 216 N. Washington Ave., Centralia, in the 5 county of Lewis and State of Washington, have invented certain new and useful Improvements in Briquets and Binders for the Same, of which the following is a specification.

10 This invention relates to binders for briquets and more particularly to a binder for briquets made of saw dust, wood fiber and the like.

The object of the invention is to provide 15 a binder of the character indicated formed of materials readily available in large quantities and at small cost and capable of producing a briquet having great density and one that will be impervious to moisture, 20 homogeneous throughout, capable of shipment and rough handling without breakage and will burn for an exceedingly long time.

Further objects and advantages of the invention will be hereinafter set forth.

25 It is a well known fact that millions of tons of saw dust go to waste, in the United States, every year. In order to utilize this otherwise waste product, I employ a binder made principally of waste products from 30 other industries and from natural vegetable matter found in great profusion and readily available and by means of this binder produce briquets of saw dust and the like, having the desirable characteristics above set 35 forth.

The aforesaid binder consists of the following ingredients, the amounts stated being such as I would use to form two tons of saw dust into briquets:

40 8 gallons of sulfite liquor, (waste liquor from paper mills).

20 pounds of gilsonite, (a well known asphalt like liquid).

45 4 gallons of a jelly derived from kelp or laminaria by macerating the natural weed and subjecting it to the action of sodium carbonate and water, preferably cold water, for twenty-four hours.

The jelly derived from the kelp is characterized by having a viscosity exceeding

that of any known substance with which I am familiar. Its viscosity far exceeds that of gum arabic or well boiled wheat starch.

In forming briquets with this binder the saw dust, or other wood pulp or wood fiber, 51 is subjected to heat until it is not only dry but is charred. It is then mixed with the binder while the latter is maintained in a heated condition and, preferably, while the saw dust is still in its heated condition. 56 When the whole has been reduced, by mixing, to an entirely homogeneous mass, it is compressed into the form of briquets in any suitable type of press, under great pressure.

These briquets dry rapidly, become exceedingly hard, will not break under handling in shipment, are impervious to moisture, may be stored in exposed places, without deterioration, for long periods, will ignite readily, will make a very hot fire and 70 will burn for an exceedingly long time, practically without smoke.

It is to be understood that the invention is not limited to the precise proportions set forth nor to the exact combination of ingredients recited but that it includes within its purview whatever changes fairly come within either the terms or the spirit of the appended claims.

Having described my invention, what I 80 claim is—

1. A binder for briquets consisting of the following ingredients used in substantially the proportions stated, to two tons of wood fiber, sulfite liquor 8 gallons, gilsonite 20 85 pounds, a jelly derived from kelp, 4 gallons.

2. The herein described process of forming briquets of saw dust, which consists of subjecting the saw dust to the action of heat to char the same, and then mixing said charred saw dust, while still in its original heated condition, with a preheated binder consisting of, substantially, to two tons of saw dust; waste sulfite liquor 8 gallons, gilsonite 20 pounds and a jelly derived from 90 kelp 4 gallons, and then compressing the mixture into briquets.

In testimony whereof I hereunto affix my signature.

LUCIUS A. KINGKINNEY.